

# United States Patent Office.

HENRY BROOK WOODCOCK, OF LOW MOOR, ENGLAND.

*Letters Patent No. 93,385, dated August 3, 1869.*

---

## IMPROVED LOW-GRADE STEEL FOR AXLES, TIRES, &c.

---

The Schedule referred to in these Letters Patent and making part of the same.

---

*To all whom it may concern:*

Be it known that I, HENRY BROOK WOODCOCK, of Low Moor, Yorkshire, England, have invented a new and useful Improvement in the Process of Manufacturing an Improved Quality of Iron, adding greatly to its capacity to resist wear, and giving to it the nature of steel, suitable for the rails for railroads, tires for locomotive-wheels, and other purposes.

My invention consists in adding to the raw pig-iron, in the process of puddling, from one-tenth ( $\frac{1}{10}$ ) to one-sixth, ( $\frac{1}{6}$ ) in weight, of ordinary blistered steel, to the weight of pig-iron. The steel does not become liquid with the iron, but, when taken out with the puddled ball adheres to it in small pieces, of the sizes originally introduced, and, in that condition, the mass is brought under a heavy hammer. The steel becomes firmly incorporated with the iron, and gives to the whole the nature of low steel, sufficient to greatly increase the wearing-surface of any article manufactured of it, especially to rails and locomotive-tires.

My said process is worked in the ordinary puddling-furnace during the process of converting pig, and, just before the charge comes to nature, a certain quantity of blistered steel, varying in proportion from about one-tenth ( $\frac{1}{10}$ ) to one-sixth, ( $\frac{1}{6}$ ), in weight, of the mass of iron with which it is to be incorporated, is thrown into the charge, and the whole puddled together.

The steel should be cut into small pieces, and, when

charged into the furnace, the pieces should be equally distributed or mixed with the iron in the puddling-furnace, so as to insure the mass being homogeneous. And although I have stated that the proportion of steel should be from one-tenth ( $\frac{1}{10}$ ) to one-sixth, ( $\frac{1}{6}$ ) in weight, of the mass of iron, those proportions giving the various grades required, I do not wish to be understood as limiting my claim of invention to those proportions.

The steel thus mixed with the pig or refined metal, either during its first or second stage of being worked, may be of any suitable kind; but blistered steel is preferable. It is worked or balled up with the iron, which may be done by any puddler in the ordinary process of puddling, and it will give to the iron the improved qualities hereinbefore named.

What I claim as my invention, and desire to secure by Letters Patent, is—

The process, substantially as herein described, of manufacturing metal possessing the qualities hereinbefore described, by mixing steel with crude iron in the process of puddling, substantially as herein described.

HENRY BROOK WOODCOCK.

Witnesses:

W. B. LANG, }  
W. NUGENT SMYTH, } Low Moor.